

3,748,271

## METHOD FOR PRODUCING ORTHOFERRITE SINGLE CRYSTALS

Hiroshi Makino, Susumu Nakamura, Takashi Okada, and Koichi Matsumi, Tokyo, Japan, assignors to Nippon Electric Company, Limited, Tokyo, Japan  
No Drawing. Filed Mar. 31, 1971, Ser. No. 129,952  
Claims priority, application Japan, Aug. 5, 1970,  
45/67,983

Int. Cl. C04b 35/40; B01j 17/18  
U.S. Cl. 252—62.57 6 Claims

## ABSTRACT OF THE DISCLOSURE

Orthoferrite single crystals are produced by first producing an orthoferrite polycrystalline body having an  $Fe_2O_3$  content ranging from about 49.8 mol percent to 50.4 mol percent and then subjecting said body to a floating-zone method in oxygen at a pressure ranging from 1 to 10 atmospheres.

The present invention relates to a method of preparing orthoferrite single crystals by the floating-zone method.

The chemical formula of orthoferrite is  $RFeO_3$  where-  
in R denotes an element selected from the group consist-  
ing of yttrium and rare earth elements. Complex ortho-  
ferrite, such as of the formula  $R_{1-x}R'_xFeO_3$ , wherein R  
and R' both denote yttrium or one of rare earth elements  
and which is obtainable by replacing a part x of R in  
 $RFeO_3$  with another element R', is meant to be included  
in the term "orthoferrite." Recent uses of orthoferrite  
single crystals have been in cylindrical domain device  
applications.

Various methods, such as the flux method and hydro-  
thermal synthesis, are known for producing orthoferrite  
single crystals. However, with such methods, the growth  
of single crystals is too slow and large single crystals are  
not obtainable. It would be desirable to provide a floating-  
zone method for producing large single orthoferrite  
crystals.

It is known that single crystals may be produced by the  
floating-zone method, providing that the object compound  
crystallizes as a solid phase congruently. This requirement  
is satisfied by orthoferrites of stoichiometric composition,  
that is, consisting of 50 mol percent  $Fe_2O_3$  and 50 mol  
percent  $R_2O_3$ .

Where the compositions of orthoferrites are slightly  
different from the stoichiometric composition and tend to-  
wards an excess of the iron component or an excess of  
the rare earth component, the floating-zone method is  
hardly useful in the manufacture of single crystals there-  
of. Since marked or significant changes in magnetic do-  
main structure and other magnetic properties of the single  
crystal do not readily occur, it is possible to employ  
single crystals of such compositions in practical applica-  
tions. Generally, when the composition varies from the  
stoichiometric composition, gas bubbles develop in or de-  
rive from the molten zone, as will be discussed later, such  
that a stable molten zone is not formed. This interrupts  
the stable growth of single crystals. In addition, numerous  
spherical pores remain in the single crystal grown under  
such conditions. Thus, a homogeneous single crystal is not  
obtainable with such compositions.

Because of the foregoing problems, it is generally re-  
quired that the polycrystalline raw material employed for  
producing a single crystal be stoichiometric in composi-  
tion. However, this has economic disadvantages in com-  
merce insofar as yield and productive efficiency are con-  
cerned.

Generally speaking, iron oxides and oxides of yttrium  
and other rare earth metals (including the metal salts and

metal hydroxides which are capable of being converted  
into oxides at higher temperatures) used as starting ma-  
terials for making orthoferrites are usually hygroscopic  
and difficult to control with regard to the metallic con-  
tents thereof. Moreover, it is difficult to regulate amounts  
of iron picked up in ball mills and other impurities which  
are absorbed in the process of preparing a polycrystalline  
raw material. Therefore, it is very difficult to prepare  
polycrystalline raw material of homogeneous composition

5 in which the molar ratio of  $Fe_2O_3$  to  $R_2O_3$  has the de-  
sired stoichiometry. The actual composition usually falls  
within the range of  $50 \pm 0.5$  mol percent of  $Fe_2O_3$ . When  
a single crystal is prepared according to the floating-zone  
10 method from polycrystalline raw material whose compo-  
sition varies or deviates to some extent from the stoichio-  
metric composition, then bubbles are formed depending  
upon the amount of deviation from the stoichiometric  
15 composition within the molten zone, the bubbles there-  
after coagulating and gradually growing into large  
bubbles in the molten zone. Finally, they escape from the  
molten zone and vanish. When this process is repeated in  
20 the course of the crystal growth, the molten zone which  
should otherwise be stable undergoes shock and, in ex-  
treme cases, the molten zone is broken.

25 It is therefore an object of the present invention to  
provide a method of making homogeneous orthoferrite  
single crystals by the floating-zone technique at an im-  
proved yield rate, even where there are slight differences  
30 in compositions among polycrystalline raw materials and  
where the compositions of the raw materials deviate from  
stoichiometry.

According to the invention, crystal growth by the float-  
ing-zone method using polycrystalline raw material is car-  
ried out in an oxygen-containing atmosphere, e.g. air or  
35 in an atmosphere of oxygen, at one to ten atmospheric  
pressure, depending upon the deviation of the compo-  
sition of the polycrystalline raw material from the stoichio-  
metric relationship of the compound of orthoferrite.

Optimum atmosphere is determined by the compo-  
40 sition of the polycrystalline raw material. Where the raw  
material contains just 50.0 mol percent  $Fe_2O_3$ , oxygen of  
at least one atmospheric pressure (atm.) can be used.  
Where the  $Fe_2O_3$  content of the raw material deviates  
45 from 50.0 mol percent by x mol percent, oxygen having  
 $(20|x|-1)$  or more atmospheric pressure should be used  
as an atmosphere during crystal growth by the floating-  
zone method using the raw material. However, the pres-  
sure should not exceed 10 atmospheres as oxygen pres-  
50 sure more than 10 atmospheres often produces an abnor-  
mal projection in part of polycrystalline raw material in  
contact with the molten zone and makes the molten zone  
unstable. Therefore pressures above 10 atmospheres  
should be avoided. Furthermore, if the deviation of the  
55 composition of polycrystalline raw material is so large  
that the  $Fe_2O_3$  content thereof lies outside the range of  
49.8 mol percent to 50.4 mol percent, then a different  
phase other than orthoferrite may tend to deposit. There-  
fore, compositions outside the foregoing range should be  
60 avoided.

According to the invention, by utilizing a single crystal  
growth furnace for the floating-zone method in which the  
atmosphere is optionally controllable, the yield rate in  
the manufacture of such crystals is markedly improved.

65 As illustrative of the invention, the following preferred  
embodiments are given.

## EMBODIMENT 1

Feed rods of polycrystalline raw materials of  $YFeO_3$   
70 were prepared by the usual method of making ferrite cer-  
amics. A feed rod was placed in a floating-zone appa-  
ratus. A molten zone was formed between the feed rod

and a seed crystal by heating to a temperature above the melting point (about 1700° C.) of  $\text{YFeO}_3$ , and the zone moved upward at a constant rate. The feed rod and the seed crystal were rotated at 30 r.p.m. in the opposite direction in order to produce a good stirring action and reduce temperature gradients. The direction of growth was generally parallel to the c-axis.

Experiments on crystal growth of  $\text{YFeO}_3$  were carried out in an oxygen atmosphere having oxygen pressures of 1 to 10 atm. and at a growth rate of about 10 mm./hr. by using feed rods having compositions of 49.5 to 50.7 mol percent  $\text{Fe}_2\text{O}_3$ . Experimental results particularly relating to gas bubble derivation from the molten zone and other phase precipitation in the crystals are shown in Table 1.

TABLE 1

| Sample number | Composition <sup>1</sup>              |                                      | Oxygen pressure (atm.) | Gas bubble derivation <sup>2</sup> | Other phase precipitation <sup>2</sup> |
|---------------|---------------------------------------|--------------------------------------|------------------------|------------------------------------|----------------------------------------|
|               | $\text{Fe}_2\text{O}_3$ (mol percent) | $\text{Y}_2\text{O}_3$ (mol percent) |                        |                                    |                                        |
| 1             | 49.5                                  | 50.5                                 | 1                      | Yes                                | Yes                                    |
| 2             | 49.5                                  | 50.5                                 | 10                     | Yes                                | Yes                                    |
| 3             | 49.8                                  | 50.2                                 | 1                      | Yes                                | No                                     |
| 4             | 49.8                                  | 50.2                                 | 3                      | No                                 | No                                     |
| 5             | 50.1                                  | 49.9                                 | 1                      | No                                 | No                                     |
| 6             | 50.1                                  | 49.9                                 | 10                     | No                                 | No                                     |
| 7             | 50.3                                  | 49.7                                 | 1                      | Yes                                | No                                     |
| 8             | 50.3                                  | 49.7                                 | 4                      | Yes                                | No                                     |
| 9             | 50.3                                  | 49.7                                 | 6                      | No                                 | No                                     |
| 10            | 50.3                                  | 49.7                                 | 10                     | No                                 | No                                     |
| 11            | 50.4                                  | 49.6                                 | 5                      | Yes                                | No                                     |
| 12            | 50.4                                  | 49.6                                 | 7                      | No                                 | No                                     |
| 13            | 50.7                                  | 49.3                                 | 1                      | Yes                                | Yes                                    |
| 14            | 50.7                                  | 49.3                                 | 10                     | Yes                                | Yes                                    |

<sup>1</sup> Composition is that of feed rod before sintering and determined by the chemical analysis.

<sup>2</sup> Yes denotes that the phenomena were more or less observed and No denotes not observed.

As will be seen from Table 1, gas bubble derivation decreases with the decrease of the deviation of feed rod composition from stoichiometry and with the increase of oxygen pressure. In the case of nearly stoichiometric composition (Sample Nos. 5 and 6), no gas bubble derivation was observed, whether under 1 oxygen atmospheric pressure or under a higher oxygen pressure of ten atmospheres whereby smooth crystal growth was obtained. Where the  $\text{YFeO}_3$  feed rod has an excess  $\text{Fe}_2\text{O}_3$  content by about 0.3 mol percent above stoichiometry (Sample Nos. 7 to 10), gas derivatives from the molten zone under 1 atmosphere, while gas derivation does not occur under a higher oxygen pressure of 6 atm. or more. Where the deviation increases up to 0.4 mol percent  $\text{Fe}_2\text{O}_3$  excess (Sample

45

phases can be produced if  $x$  satisfies the relationship  $-0.2 \leq x \leq 0.4$ . In this case, if  $|x| \leq 0.1$ , no gas bubble is derived from the molten zone under 1 atm. oxygen pressure. If  $|x| > 0.1$ , no gas bubble derivation occurs under an oxygen pressure of  $(20|x| - 1)$  atmospheres or more.

Although the growth rate was 10 mm./hr. in the above experiments, results did not vary under a growth rate of 3 mm./hr. to 20 mm./hr.

## EMBODIMENT 2

By using the same technique as Embodiment 1, single crystals of  $\text{TbFeO}_3$ ,  $\text{ErFeO}_3$  and  $\text{YbFeO}_3$  were grown. Typical results are shown in Table 2. High oxygen pressure of  $20|x| - 1$  or more atmospheres is also effective in these cases, as is seen from Table 2.

TABLE 2

| Sample number | Composition <sup>1</sup>              |                                      | Oxygen pressure (atm.) | Gas bubble derivation <sup>2</sup> | Other phase precipitation <sup>2</sup> |
|---------------|---------------------------------------|--------------------------------------|------------------------|------------------------------------|----------------------------------------|
|               | $\text{Fe}_2\text{O}_3$ (mol percent) | $\text{R}_2\text{O}_3$ (mol percent) |                        |                                    |                                        |
| 15            | 50.2                                  | $\text{Tb}_2\text{O}_3$ , 49.8       | 1                      | Yes                                | No                                     |
| 16            | 50.2                                  | $\text{Tb}_2\text{O}_3$ , 49.8       | 7                      | No                                 | No                                     |
| 17            | 50.3                                  | $\text{Er}_2\text{O}_3$ , 49.7       | 1                      | Yes                                | No                                     |
| 18            | 50.3                                  | $\text{Er}_2\text{O}_3$ , 49.7       | 8                      | No                                 | No                                     |
| 19            | 49.9                                  | $\text{Yb}_2\text{O}_3$ , 50.1       | 1                      | No                                 | No                                     |
| 20            | 50.3                                  | $\text{Yb}_2\text{O}_3$ , 49.7       | 1                      | Yes                                | No                                     |
| 21            | 50.3                                  | $\text{Yb}_2\text{O}_3$ , 49.7       | 7                      | No                                 | No                                     |

NOTE.—See footnotes 1 and 2 at end of Table 1.

## EMBODIMENT 3

Sample Nos. 22 to 24 of Table 3 show that the invention is also effective for  $\text{YFeO}_3$  in which Fe is partially replaced with  $\text{Co}^{3+}$ . Since Co occupies the site of Fe in the crystal lattice, the stoichiometric composition of the raw material in this case is 50 mol percent  $\text{Y}_2\text{O}_3$  and 50 mol percent in total of  $\text{Fe}_2\text{O}_3$  plus  $\text{Co}_2\text{O}_3$ .  $\text{Co}^{3+}$  may replace up to 5 atomic percent of Fe. Sample No. 25 of Table 3 represent that the invention can be successfully applied to production of  $\text{YFeO}_3$  in which part of Fe is replaced with  $\text{Co}^{2+}$  and  $\text{Ti}^{4+}$ . Since Co and Ti occupy the sites of Fe ions in the crystal, the stoichiometric composition of the raw material is 50 mol percent  $\text{Y}_2\text{O}_3$  and 50 mol percent in total of  $\text{Fe}_2\text{O}_3$ ,  $\text{CoO}$  and  $\text{TiO}_2$  in this case. Co and Ti may replace up to 5 atomic percent of Fe. Where the feed rod composition  $\text{Fe}_2\text{O}_3 + \text{Co}_2\text{O}_3$  or



is  $50+x$  mol percent, the floating-zone melting under an oxygen pressure of  $20|x| - 1$  atm. or more can produce good single crystals.

TABLE 3

| Sample number | Composition <sup>1</sup> (mol percent) |                                   |                        | Oxygen pressure (atm.) | Gas bubble derivation <sup>2</sup> | Other phase precipitation <sup>2</sup> |
|---------------|----------------------------------------|-----------------------------------|------------------------|------------------------|------------------------------------|----------------------------------------|
|               | $\text{Fe}_2\text{O}_3$                | $\text{Co}_2\text{O}_3$           | $\text{Y}_2\text{O}_3$ |                        |                                    |                                        |
| 22            | 49.8                                   | 0.3                               | 50.0                   | 1                      | No                                 | No                                     |
| 23            | 50.1                                   | 0.3                               | 49.6                   | 1                      | Yes                                | No                                     |
| 24            | 50.1                                   | 0.3                               | 49.6                   | 10                     | No                                 | No                                     |
| 25            | 49.8                                   | $\text{CoO} + \text{TiO}_2$ , 0.2 | 50.0                   | 1                      | No                                 | No                                     |

NOTE.—See footnotes 1 and 2 at end of table 1.

Nos. 11 and 12), still high oxygen pressure of 7 atmospheres or more is necessary to stop gas bubble derivation. If the feed rod composition deviates toward the  $\text{Y}_2\text{O}_3$  excess side by 0.2 mol percent from the stoichiometry (Sample Nos. 3 and 4), a higher oxygen pressure of 3 or more is needed. On the other hand, application of oxygen pressure cannot stop gas bubble derivation and precipitation of other phases than orthoferrite in the resultant single crystal, if the deviation of the composition is too large (Sample Nos. 1, 2, 13 and 14).

The deviation of feed rod composition from the stoichiometry and the oxygen pressure necessary to stop the gas bubble derivation appears to have nearly a linear relationship. Summarizing the foregoing, where the  $\text{Fe}_2\text{O}_3$  composition of polycrystalline raw material is expressed by  $50+x$  mol percent, single crystals having no other

Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and the appended claims.

What is claimed is:

1. A method of producing orthoferrite single crystals comprising the steps of preparing an orthoferrite polycrystalline body consisting essentially of  $\text{Fe}_2\text{O}_3$  and one oxide selected from the group of  $\text{Y}_2\text{O}_3$ ,  $\text{Tb}_2\text{O}_3$ ,  $\text{Er}_2\text{O}_3$ , and  $\text{Yb}_2\text{O}_3$ , the  $\text{Fe}_2\text{O}_3$  content being  $50+x$  mol percent with  $x$  ranging from  $-0.2$  to  $+0.4$ , and subjecting said polycrystalline body to floating zone melting by heating said

polycrystalline body at a temperature higher than the melting point of said polycrystalline body to form a molten zone between said polycrystalline body and a seed crystal and moving said molten zone at a rate of 3 to 20 mm. per hour in an oxygen atmosphere having a pressure of at least one atmospheric pressure where  $|x| \leq 0.1$  and at least  $20|x|-1$  atmospheric pressure where  $|x| > 0.1$ , the pressure of said atmosphere being not more than ten atmospheric pressure.

2. The method claimed in claim 1, in which the oxide is  $\text{Y}_2\text{O}_3$ .

3. A method of producing orthoferrite single crystals comprising the steps of preparing an orthoferrite polycrystalline body consisting essentially of  $\text{Fe}_2\text{O}_3$  and one oxide selected from the group of  $\text{Y}_2\text{O}_3$ ,  $\text{Tb}_2\text{O}_3$ ,  $\text{Er}_2\text{O}_3$ , and  $\text{Yb}_2\text{O}_3$ , wherein an amount ranging up to 5 atomic percent of Fe is replaced by  $\text{Co}^{3+}$  as  $\text{Co}_2\text{O}_3$ , and wherein the  $\text{Fe}_2\text{O}_3$  and the  $\text{Co}_2\text{O}_3$  content is  $50+x$  mol percent with  $x$  ranging from -0.2 to +0.4, and subjecting said polycrystalline body to floating zone melting by heating said polycrystalline body at a temperature higher than the melting point of said polycrystalline body to form a molten zone between said polycrystalline body and a seed crystal and moving said molten zone at a rate of 3 to 20 mm. per hour in an oxygen atmosphere having a pressure of at least one atmospheric pressure where  $|x| \leq 0.1$  and at least  $20|x|-1$  atmospheric pressure where  $|x| > 0.1$ , the pressure of said atmosphere being not more than ten atmospheric pressure.

4. The method claimed in claim 3, in which the oxide is  $\text{Y}_2\text{O}_3$ .

5. A method of producing orthoferrite single crystals comprising the steps of preparing an orthoferrite polycrystalline body consisting essentially of  $\text{Fe}_2\text{O}_3$  and one

oxide selected from the group of  $\text{Y}_2\text{O}_3$ ,  $\text{Tb}_2\text{O}_3$ ,  $\text{Er}_2\text{O}_3$ , and  $\text{Yb}_2\text{O}_3$ , wherein an amount ranging up to 5 atomic percent of Fe is replaced by a combination of  $\text{Co}^{3+}$  and  $\text{Ti}^{4+}$  as  $\text{CoO}$  and  $\text{TiO}_2$  and wherein the  $\text{Fe}_2\text{O}_3$ , the  $\text{CoO}$  and the  $\text{TiO}_2$  content is  $50+x$  mol percent with  $x$  ranging from -0.2 to +0.4, and subjecting said polycrystalline body to floating zone melting by heating said polycrystalline body at a temperature higher than the melting points of said polycrystalline body to form a molten zone between said polycrystalline body and a seed crystal and moving said molten zone at a rate of 3 to 20 mm. per hour in an oxygen atmosphere having a pressure of at least one atmospheric pressure where  $|x| \leq 0.1$  and at least  $20|x|-1$  atmospheric pressure where  $|x| > 0.1$ , the pressure of said atmosphere being not more than ten atmospheric pressure.

6. The method claimed in claim 5, in which the oxide is  $\text{Y}_2\text{O}_3$ .

#### References Cited

##### UNITED STATES PATENTS

|           |         |                     |             |
|-----------|---------|---------------------|-------------|
| 3,272,591 | 9/1966  | Rudness et al. ---  | 252—62.57 X |
| 3,414,372 | 12/1968 | Paulus et al. ----- | 23—51 R     |
| 3,485,759 | 12/1969 | Kolb et al. -----   | 252—62.57   |

##### OTHER REFERENCES

Plaskett et al., "IBM Technical Disclosure Bulletin," vol. 13, No. 9, p. 2632, February 1971.

OSCAR R. VERTIZ, Primary Examiner  
J. COOPER, Assistant Examiner

##### U.S. CL. X.R.

252—62.56, 62.59; 423—263, 594; 23—301 SP